

## UNITED STATES PATENT OFFICE

2,520,105

## METACHROME DYEING PROCEDURE

Henry E. Millson, Plainfield, and Chester A. Amick and Willard H. Watkins, Bound Brook, N. J., assignors to American Cyanamid Company, New York, N. Y., a corporation of Maine

No Drawing. Application May 27, 1947,  
Serial No. 750,886

10 Claims. (Cl. 8—30)

1

This invention relates to improved metachrome dyeing processes.

In the past there have been four general procedures employed in dyeing with metallizable dyes. The first utilizes preformed metallized dyes and requires the formation of the metallized dye before it is introduced into the dye bath. Practically all of the metallizable dyes may be utilized in this process, but it is subject to a number of disadvantages. The dye is not very efficiently used, the dye bath is poorly exhausted, and the color value is not as high as desirable in some cases.

The second process is referred to as an "after chrome" or "top chrome" procedure in which the fabric is dyed with metallizable dyes and then subjected to an after treatment with a solution of a compound of the metal to be introduced into the dye molecule. As the name implies, the dye is applied the same as an acid dye, and it requires an extra process and extra time for the formation of the metallized complex.

The third procedure is the so-called "bottom chrome" process in which a metal compound is first deposited in the textile fiber and then the dye is applied and the metallized complex forms in the fiber. Here again this process is an extremely long one requiring several steps.

The fourth procedure is the so-called metachrome process in which the metallizable dye and the compound of the metal to be introduced are both present in the dye bath at the start and the metallized dye is formed both in the fiber and in the bath itself and not introduced as a preformed compound.

The metachrome process presents many advantages. However, in many cases the dye is not effectively utilized when dyeing basic nitrogenous fibers such as the natural animal fibers, wool, silk, and the like or synthetic fibers of similar type from casein, polyamides, and so forth. Certain dyes give good uniform fiber penetration in a yarn, and others penetrate only some of the fibers. The dyes which do not penetrate all of the fibers or are destroyed during the dyeing operation, particularly in the case of heavier shades, have, therefore, been considered unsuitable for use in the metachrome process and have required resort to the process starting out with the preformed metallized dye or the top or bottom chrome processes with their attendant disadvantages.

According to the present invention it is found that markedly increased strength and levelness of

2

dyeing is obtained if three factors are present in the process. These three factors are:

1st: The presence of a salt of an alkaline earth metal.

5 2nd: A water dispersible surface active composition containing at least one cationic surface active agent.

10 3rd: The pH of the dye bath is sufficiently high initially so that rapid chromation is prevented or retarded, and during the dyeing process the pH is progressively lowered until final chromation results.

15 With certain dyes any one of the three factors referred to above will effect some improvement either in color value or levelness, but with certain other dyes, both of these improvements in dyeing characteristics are not obtained with metallizable dyes unless all three of the above reaction conditions are present, and the present 20 invention contemplates only processes in which all three factors are effective.

25 The alkaline earth metal salts or salts to be used are not in the least critical. Any of the common soluble salts may be used. The different alkaline earth metal salts will vary to some extent in their effect, and this variation is not the same with all metallizable dyes. In general, best results are obtained with magnesium salts, magnesium sulfate being particularly desirable, by 30 reason of its cheapness, ready availability and the excellent results which it gives in the process of the present invention. Accordingly magnesium sulfate represents the preferred alkaline earth metal salt, though in its broader aspects the invention is not limited to its use.

35 The reason for the improved results obtainable with alkaline earth metal salts, and particularly the increased strength of dyeing which follows their use, has not been completely determined and, therefore, the present invention is 40 not intended to be limited to any theory of the action of the alkaline earth metal salts. Certain observations with certain dyestuffs make it appear very probable, that at least with some dyestuffs, magnesium or the other alkaline earth metal salts actually form metal complexes with the dye, which complexes are only stable in solutions of high pH. Some of the dyes change their color very strikingly when they are introduced 45 into a dye bath containing the alkaline earth metal salt. Such a great change in color, which is again reversed as the dyeing proceeds and the pH fails to sufficiently low values, makes it almost certain that there is an actual chemical 50 change in the dye molecule. The conditions un-

der which this color change takes place with some of the metallizable dyes make it probable that the alkaline earth metal salt actually forms a dye complex which is then decomposed when the pH falls to a sufficiently low value. This explanation is consistent with the relatively strong basic character of the alkaline earth metal salt which would make it probable that if a complex is formed, it would not be acid stable. The above explanation is advanced, therefore, as probable in the case of some at least of the metallizable dyes which may be used in the process of the present invention.

It is an advantage of the invention that the amount of the added alkaline earth metal salts is not critical. It should, however, be realized that the action appears to be in no sense catalytic. Relatively substantial amounts of alkaline earth metal salt must be added. Normally the amount added is at least equal to the weight of the dye, although this figure does not represent a sharp or critical dividing line. Smaller amounts will exert an effect, but one which rapidly diminishes as the amount of salt becomes inadequate. It has been found that the amount of alkaline earth metal salt may be advantageously correspondingly greater than the weight of the dyestuff. For example, the use of five times as much alkaline earth metal salt gives excellent results, and since the alkaline earth metal salts are relatively cheap chemicals, it is preferred to use them in excess of the weight of the dyestuff, although the invention is not broadly limited to this preferred amount.

The second factor requires a water dispersible surface active composition containing at least one cationic surface active agent. It is also desirable that any insoluble reaction products of the cationic surface active agent be likewise dispersible. This dispersibility of the surface active composition may be effected in several ways. For instance, the cationic surface active agent may be colloidized either by itself or in combination with the dyestuff or alkaline earth metal salt or with the chromating mordant. These methods are described in Patent No. 2,434,178 issued January 6, 1948 to Royer and Amick. Another method of obtaining water dispersibility is to associate the cationic surface active agent with nonionic surface active agents as is described in the Milson and Royer application Serial No. 420,504, filed November 26, 1941.

The present invention is not concerned with the particular methods of achieving dispersibility of the surface active component, this forming the subject matter of the applications above referred to. On the contrary, the present invention is concerned only with water dispersible cationic surface active compositions when associated with the other two factors of the process of the present invention, namely, the presence of the alkaline earth metal salt and the initial high pH of the dye bath.

The third factor, namely, high initial pH, is also not a critical operating procedure. It will vary quite widely with different dyestuffs and with different fabrics. In general it will never be lower than 5.5 and the upper limit is from about 8 to 9.5. The upper limit is defined, not so much by the reaction itself, as by the fabric, because it is necessary to maintain the pH below the point at which the basic nitrogenous fibers are injured. In general, the initial pH should be chosen sufficiently high to retard initial chro-

mation. With dyestuffs with which it seems probable that a complex is formed with the alkaline earth metal salt, the pH initially should be high enough so that the complex, if there be one present, is not decomposed until the dyeing of the fiber has proceeded to the desired extent.

As the fibers are dyed and the normal heating of the bath continues, there is a definite lowering of pH, the bath becoming more and more acid. When the pH gets low enough, both dyeing and chromation proceed more rapidly, and a final dyeing of high strength and good levelness results. Thus it is now possible to obtain deep shades, such as a deep chrome black, by a true metachrome process.

While, as pointed out above, the pH of the dye bath is lowered by the dyeing procedure itself, probably because of a reaction of the basic nitrogenous fiber with the alkali present, this lowering is usually insufficient, hence in the majority of cases it is desirable to add small amounts of acid or acid salts as the dyeing proceeds. Preferably the acid is added in parts— $\frac{1}{2}$  after one-half hour boiling, and  $\frac{1}{2}$  after an hour's boiling. The exact amount of addition of acid and the time and portions are not critical, but optimum results will vary a little with different colors. This is entirely consistent with normal dyeing practice where it is usually necessary to make some changes in the dyeing time, temperature, and pH with different dyes and different fibers in order to get the best results. The same type of adjustment is employed in the process of the present invention which is an advantage as the dyer does not have to learn new techniques.

While the process of the present invention gives important improvement in dyeing with ordinary dyes by the metachrome method, producing strong shades with a high degree of levelness and excellence of fastness to light and washing, a further advantage lies in the fact that certain chromable dyes, which are dyeable in the metachrome process only when the wool has been modified by one of the various non-felting treatments, such as chlorination, can be dyed by the present process on ordinary wool. This is important as it opens up a new field for these dyes. In addition to the improved results obtained by the process of the present invention, a further advantage lies in the material saving which can be effected in the amount of chromium containing salt used. In favorable cases this may amount to 40 or 50%.

The invention will be described in greater detail in conjunction with the following specific examples. The parts are by weight.

#### Example 1

One part of the condensation product of octadecyl guanidine bicarbonate and ethylene oxide (1 mole to 6 moles) are dissolved in an excess of organic solvent, e. g., ether. 20 parts of Epsom salts are added and the ether evaporated slowly with constant stirring to deposit the cationic agent on the Epsom salts base. Finally the product is vacuum dried. When the drying is completed, the product is grindable. 52.5 parts of this product is dry-blended with 3 parts of powdered  $K_2Cr_2O_7$  to give a mordant. Twelve percent of this product (based on the weight of the wool) is used with 2% of the ordinary commercial chrome types to give a satisfactory dyeing. The dyeing is made as follows:

75 2% dye (C. I. 202) predispersed in boiling

water was admixed with 12% of the mordant and a sufficient amount of ammonia or ammonia and ammonium salt such as ammonium dihydrogen phosphate, to produce a pH of about 8.5 to 9.0 in a 400 cc. volume, sufficient water being used to make the necessary dilution.

A 5 gram woolen piece or skein is pre-wet with water and entered into the dye bath at 120° F. The dye liquor is gradually brought to the boil in  $\frac{1}{2}$  hour with frequent turning of the wool to insure uniform dyeing. Boiling and turning are continued for  $\frac{1}{2}$  hour, after which 2% of 28% acetic acid is added. After another half-hour on the boil, 4% of 28% acetic acid is added. Dyeing is continued at the boil for a third half-hour making a total dyeing time of two hours. The color of the dyed skein is blue-black and the dyeing has good fastness and is very level. Ordinarily this color can be dyed satisfactorily only by the very cumbersome top or bottom chrome method.

*Example 2*

37.5 parts of corn dextrine made by dextrinizing corn starch with hydrochloric acid, 37.5 parts of Epsom salts, 3.75 parts of the cationic agent of Example 1, 4.5 parts of  $K_2Cr_2O_7$  and about 20 parts of water are wet-blended in a Werner-Pfleiderer mixer until uniform. This gives a thick plastic magma. The product is then transferred to enameled trays and dried in a vacuum dryer, ground and screened through a 140 mesh screen. 12% of this product is substituted for the material in Example 1 and dyeings are carried out in the same way with essentially the same results.

The chrome equivalent amount of  $K_2CrO_4$  can be used in place of the  $K_2Cr_2O_7$ .

*Example 3*

The product of Example 2 is used in making a dyeing of the dye C. I. 652, using the dyeing formula of Example 1. This dye gives an excellent color value which is superior to that obtained by ordinary metachrome dyeings or even top chrome dyeings.

*Example 4*

500 parts of the dextrine of Example 2 and 100 parts of the condensation product of octadecyl guanidine bicarbonate and ethylene oxide (1 mole to 6 moles) are blended in a Werner-Pfleiderer mixer with sufficient water to give a stiff plastic magma. The well mixed material is then transferred to enameled trays and vacuum dried. It is then ground and screened through a 140 mesh screen. 30 parts of this product, 24 parts of 100 mesh Epsom salts, and 6 parts of 140 mesh  $K_2Cr_2O_7$  are dry-blended to give a mordant. 6% of this mordant and 2% of 28%  $NH_4OH$  (both on the weight of the wool) and 100 mg. of the dye having C. I. 203 are dyed on a 5 gram woolen skein as in Example 1. The dyeing obtained is blue-black, has excellent fastness properties and is fiber level.

*Example 5*

37.5 parts of the dextrine of Example 2, 37.5 parts of Epsom salts, 3.75 parts of a condensation product of octadecyl guanidine bicarbonate and ethylene oxide (1 mole to 6 moles), 4.5 parts of potassium bichromate and about 20 parts of water are added to a Werner-Pfleiderer mixer and worked until homogeneous. A thick plastic magma is produced which is transferred to enameled trays, dried in the vacuum dryer, ground

and screened through a 140 mesh screen producing a colloidized mordant.

A dye bath is prepared as follows:

5 0.1 g. dye (C. I. 202) predispersed in boiling water, approximately 2% of 28%  $NH_4OH$  to give a pH not greater than 9.5  
12% colloidized mordant  
400 cc. dye bath volume

10 A 5 gram woolen piece or skein is pre-wet with water and entered into the dye bath at 120° F. The dye liquor is gradually brought to the boil in  $\frac{1}{2}$  hour with frequent turning of the wool to insure uniform dyeing. Boiling and turning are continued for  $\frac{1}{2}$  hour after which  $\frac{1}{3}$ % of  $H_2SO_4$  is added. Dyeing is continued at the boil for a second half hour, after which  $\frac{2}{3}$ % of  $H_2SO_4$  is added. Dyeing is then continued for a third half-hour at the boil making a total dyeing time of two hours.

15 The color of the dyed skein is blue-black and the dyeing has good fastness and is fiber level. Ordinarily this color can be dyed satisfactorily only by the very cumbersome top or bottom chrome method.

20 25 The same results are obtained if the potassium bichromate is substituted by a chromium equivalent amount of potassium chromate.

*Example 6*

30 The dyeing procedures of the preceding example is repeated using the dye C. I. 652 instead of the dye of Example 5. The dye gives an excellent color value which is superior to that obtained by ordinary metachrome dyeings or top chrome dyeings.

*Example 7*

35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9

## Example 10

2 parts of the dye C. I. 274, and one part of the condensation product of 2 mols of polyethylene oxide (molecular weight 4000), and 1 mol of the dimerized acid obtained by heat treating soya bean acids and distilling off the monomeric acids are dry blended. 3% of this product, 6% of the mordant of Example 4 and 2% of 28% ammonia are dissolved in 400 parts of water and wool is dyed therein by the procedure of Example 1. A good, bright orange color is obtained and the dyed wool has good fastness and levelness.

## Example 11

A dye bath is prepared with 1 part of the dye having the Color Index #203 (pure presscake) dispersed in 2000 parts of boiling water. This is then diluted with an equal amount of water containing 6 parts of the mordant of Example 4 and 2 parts of 28% ammonia. Fifty parts of pre-wet wool are then entered and dyed as in Example 5. A black shade of good fiber levelness is obtained.

## Example 12

The procedure of Example 4 is repeated, except the dyeing is made on synthetic casein fiber and the dye is nitro amino phenol diazotized and coupled with meta-phenylene diamine which is diazotized and coupled to 5-sulfo  $\alpha$ -naphthol, Prototype 14. An excellent brown dyeing is obtained.

## Example 13

The procedure of Example 4 is repeated, except the dye is C. I. 652 and the material is nylon. A strong, bright red shade is obtained.

## Example 14

The procedure of the preceding example is repeated except the dye is C. I. 292. A good slate green shade is obtained which is commercially satisfactory.

## Example 15

50 parts of the dextrine of Example 2 and 10 parts of the condensation product of octadecyl guanidine bicarbonate and ethylene oxide (6-1) are colloidized and vacuum dried. This product is then ground, screened through a 100 mesh screen, and dry blended with 40 parts of the commercial dye having Color Index No. 203.

A batch of woolen fabric is dyed in a commercial dye kettle as follows:

10% of the above blended color  
6% ammonium acetate  
3.3% Epsom salts  
0.7% potassium dichromate

The cloth was entered into the dye kettle, and wet out with water. If necessary, the cloth is treated to make it neutral, after which the treating water was discharged from the kettle, refilled, heated to 120° F. and the above ingredients added in the order given. The starting pH was about 5.5 as determined by Universal indicator paper. The dye liquor was slowly heated to 207° to 208° F. at which time the pH was about 6.0 and run about 40 minutes, after which 2% of 28% acetic acid was fed on and the pH dropped to 5.0. After dyeing for an additional 40 minutes, 2% of 28% acetic acid was added a second time, and the pH remained about 5.0.

When the dyeing was completed, the woolen fabric was dyed a black color having good fastness and levelness.

## Example 16

A dyeing composition is prepared by dry blending 60 parts of the colloidized cationic surface active agent of the preceding example with 5 40 parts of the yellow dyestuff prepared by diazotizing sulfanilic acid and coupling to 2-hydroxy-5-amino benzoic acid.

A dyeing is prepared as follows:

10 All weights are based upon the weight of the wool to be dyed  
5% of the blended dye prepared as in the preceding paragraph  
10% ammonium sulfate  
0.6% potassium dichromate  
Bath ratio: 80-1

The starting pH of this dye solution will vary from a pH of 5.0-6.0 depending upon the previous history of the wool and how thoroughly it has been neutralized after the preceding operation.

The bath is brought to the boil gradually in 30 minutes, boiled 30 minutes, after which 3% of the 28% acetic acid is added. After an additional 30 minutes at the boil, a second addition of 3% of 28% acetic acid is added and the boiling continued for another 30 minutes.

Wool dyed as above has a brilliant yellow color, showing excellent levelness and good fastness properties.

## Example 17

The procedure of Example 1 is repeated except the dye C. I. 1085 is used instead of C. I. 202 of Example 1. The dyeing produces a blue-black shade which is level and has excellent fastness properties.

## Example 18

A dye bath is prepared as follows, all weights being based on the wool.

2% dye having Color Index No. 202  
2% of 28% ammonium hydroxide  
1% of the non-ionic agent prepared by reacting 2 moles of poly-ethylene oxide (M. W. 4000) and 1 mole of the dimerized acid obtained by heat treating soya bean acids and distilling off the monomeric acid  
0.5% of the cationic active agent of Example No. 1  
50 10% Epsom salts  
0.6% potassium dichromate

The dye bath is then made up to 400 cc. with water, after which a 5-gram woolen piece or skein is pre-wet and dyed as in Example No. 1 or No. 5 and the strength and shade of the dyed piece is generally like that obtained from Example No. 1

## Example 19

60 The procedure of Example No. 18 is repeated except the dye having Color Index No. 652 is used instead of the dye having Color Index No. 202. Wool dyed by this color and procedure gives excellent strength and levelness, usually superior to the conventional topchrome methods of dyeing.

## Example 20

The procedure of Example No. 18 is repeated 70 except the dye having Color Index No. 98 is used in place of the dye having Color Index No. 202. Wool dyed by this color and procedure has excellent strength and fiber levelness, being equal usually to a top chrome dyeing as made by the conventional methods.

*Example 21*

The procedure of Example No. 18 is repeated except the dye having Color Index No. 1085 is used in place of the dye having Color Index No. 202. Wool dyed by this color and procedure has good color value and fiber levelness.

*Example 22*

The procedure of Example No. 18 is repeated except the dye having Color Index No. 201 is used in place of the dye having Color Index No. 202. Wool dyed by this dye and procedure is stronger and brighter than wool dyed with an equivalent amount of dye which is dyed by the conventional top chrome procedure.

*Example 23*

The procedure of Example 18 is repeated except the dye having Color Index 274 is used in place of the dye having Color Index No. 202. Wool so dyed has excellent color value, is bright and has good fiber levelness.

*Example 24*

400 parts of yellow corn dextrine and 100 parts of the cationic surface active agent described in Example 1 are intimately mixed and vacuum dried as described. 5 parts of this material are then dissolved in 95 parts of water to give a 1% solution of the cationic surface active agent. A dye bath is then prepared as follows:

2% of the dye having Color Index No. 203 pre-dissolved in 100 ml. water  
 300 ml. of water  
 2% of 28% ammonium hydroxide  
 2.5 ml. of the 1% solution of cationic surface active agent described above.  
 10% Epsom salts  
 0.6% potassium bichromate

A 5-gram pre-wet wool skein is then dyed therein, using the dyeing procedure on Example No. 1 and the strength and shade of the dyed wool is very fiber level and is usually stronger than equivalent dyeings made by the conventional top chrome procedure. Magnesium acetate or magnesium chloride may be substituted for the Epsom salts.

The addition of the ammonium hydroxide generally changes the pH to 9-9.6 depending upon the pH of the water added to the dyebath. The shade of the dye having Color Index No. 203 is plum colored or reddish after the addition of the water to make up the dyebath, particularly if distilled water having a pH lower than 7 is used. After the addition of the ammonium hydroxide, the shade of this color becomes greenish-blue. Upon the addition of the Epsom salts the color of the dye solution becomes a cherry red, although there is no appreciable change in pH. During the subsequent dyeing, this dyebath exhausts very rapidly, much more so than when a similar dyeing is made except the Epsom salts is omitted.

*Example 25*

The procedure of Example 24 is repeated, except 10% of calcium nitrate  $\frac{4}{4}$  H<sub>2</sub>O is substituted for the Epsom salts of Example 24. The shade of the dyed wool is slightly grayer than that obtained when Epsom salts is used. The addition of 10% of the calcium nitrate  $\frac{4}{4}$  H<sub>2</sub>O based on the weight of the wool to the dyebath likewise caused no appreciable change in pH but did cause the blue green shade of the dye solution to become a brighter red.

*Example 26*

The procedure of Example 24 is repeated except 10% of barium nitrate is used instead of the Epsom salts. The wool dyed from this bath is slightly bluer and brighter than that dyed by the procedure of Example 24.

*Example 27*

The procedure of Example 25 is repeated except the dye having Color Index No. 652 is used instead of the dye having Color Index No. 203. A good strong red dyeing is obtained. If desired, the calcium nitrate may be replaced with strontium chloride.

*Example 28*

The procedure of Example 18 is repeated exactly except 0.5% of the surface active agent, tertiary amine hydroacetate, prepared according to U. S. P. 2,200,815 is used instead of the surface active agent prepared by the condensation of octa decyl guanidine bicarbonate and ethylene oxide (6:1) which was used in Example 2. Wool dyed with this procedure shows good strong blue-black color with good penetration.

*Example 29*

The procedure of the preceding example is followed exactly except the surface active agent, cetyl pyridinium chloride, is used instead of the tertiary amine hydroacetate of the preceding example. A good strong bright blue-black dyeing is obtained.

*Example 30*

The procedure of the preceding experiment is repeated except the surface active agent, cetyl trimethyl ammonium bromide is used instead of the cetyl pyridinium chloride. A good strong bright blue-black dyeing is obtained.

*Example 31*

The procedure of Example 18 is repeated exactly except the surface active non-ionic agent of Example 18 is replaced by 1% of beta hydro-triethoxy-propyl-lauramide. A good bright blue-black dyeing which showed excellent penetration is obtained.

*Example 32*

The procedure of the preceding example is repeated exactly except the beta-hydro-triethoxy-propyl-lauramide is replaced with 1% of p-hexadecyl phenyl ether of polyethylene glycol.

*Example 33*

The procedure of Example 18 is repeated except the non-ionic surface active agent of Example 18 is replaced with the condensation product of stearyl alcohol with 8 moles of ethylene oxide liquified with 30% H<sub>2</sub>O. Wool dyed by this procedure gives a bright blue-black shade showing excellent penetration and good fiber levelness.

*Example 34*

The procedure of Example 18 is repeated except the non-ionic surface active agent of Example 18 is replaced with 1% of hexa-ethylene glycol dodecyl amino triazine resin. The strength obtained with this combination is not as good as with the combination of Example 18 but is much superior to the results obtained when no surface active agents are present.

In the specific examples no additional chromium compound is added during the dyeing. In the production of most shades particularly lighter

shades, this gives the best results. However, in some cases, particularly with dark shades such as maroon, brown, navy and black, it is sometimes advantageous to add small amounts of additional bichromates, for example, .3 to .5%, to the bath after it has been boiling for about one-half hour or so. The additional chromium makes the dark shades somewhat richer and in many cases improves fastness to wet finishing. The addition of small amounts of the chromates to the bath after the dyeing has proceeded for some time is therefore included in the scope of the present invention.

The improved results obtainable by means of the present invention are not always the same with each dye. In many cases improved strength and penetration result; in other cases, the levelness is better while with some dyes, improvements in both characteristics are observed. The degree of improvement in various characteristics varies with the dye. In general, the process of the present invention shows less marked advantages with some yellow dyes than with dyes of other shades.

In the examples, dyestuff mixtures have been colloidized by working in a relatively stiff paste with carbohydrates such as dextrine and dried at a low temperature so that the individual particles on contact with water dispersed rapidly without violent agitation to form a colloidal solution. Such products have been described in the specification as "colloidized." This term is used in the claims in no other sense.

We claim.

1. A method of dyeing which comprises subjecting substantially unmetallized basic nitrogenous fibers to the action of a dye bath formed by mixing a chromable dye, a soluble chromium containing salt, a soluble alkaline earth metal salt, a water-dispersible surface-active composition containing at least one cationic surface active agent, water, and sufficient alkali to make the bath alkaline and to cause said dye to react with said alkaline earth metal salt to form an alkaline earth metal complex of said dye and insufficient to materially damage the fibers, partially dyeing said fibers from said complex, gradually lowering the pH of said bath to a point where decomposition of said complex and chromation take place, and completing the dyeing at said lowered pH.

2. A method of dyeing which comprises subjecting substantially unmetallized basic nitrogenous fibers to the action of a dye bath formed by mixing a chromable dye, a soluble chromium containing salt, magnesium sulfate, a water-dispersible surface-active composition containing at least one cationic surface active agent, water, and sufficient alkali to make the bath alkaline and to cause said dye to react with said alkaline earth metal salt to form an alkaline earth metal complex of said dye and insufficient to materially damage the fibers, partially dyeing said fibers from said complex, gradually lowering the pH of said bath to a point where decomposition of said complex and chromation take place, and completing the dyeing at said lowered pH.

3. A method of dyeing which comprises subjecting substantially unmetallized basic nitrogenous fibers to the action of a dye bath formed by mixing a chromable dye, a soluble chromium containing salt, a soluble alkaline earth metal salt, a water-dispersible surface-active composition containing at least one cationic surface active agent, water, and sufficient alkali to make

the bath alkaline and to cause said dye to react with said alkaline earth metal salt to form an alkaline earth metal complex of said dye and insufficient to materially damage the fibers, partially dyeing said fibers from said complex, gradually lowering the pH of said bath by the addition of successive small portions of acid to a point where decomposition of said complex and chromation take place, and completing the dyeing at said lowered pH.

4. A method of dyeing which comprises subjecting substantially unmetallized basic nitrogenous fibers to the action of a dye bath formed by mixing a chromable dye, a soluble chromium containing salt, magnesium sulfate, a water-dispersible surface-active composition containing at least one cationic surface active agent, water, and sufficient alkali to make the bath alkaline and to cause said dye to react with said alkaline earth metal salt to form an alkaline earth metal complex of said dye and insufficient to materially damage the fibers, partially dyeing said fibers from said complex, gradually lowering the pH of said bath by the addition of successive small portions of acid to a point where decomposition of said complex and chromation take place, and completing the dyeing at said lowered pH.

5. A method of dyeing which comprises subjecting substantially unmetallized basic nitrogenous fibers to the action of a dye bath formed by mixing a chromable dye, a soluble chromium containing salt, a soluble alkaline earth metal salt, a water-dispersible surface-active composition containing at least one cationic surface active agent, water, and sufficient alkali to make the bath alkaline, but with a pH not greater than 9.5, and to cause said dye to react with said alkaline earth metal salt to form an alkaline earth metal complex of said dye and insufficient to materially damage the fibers, partially dyeing said fibers from said complex, gradually lowering the pH of said bath to a point where decomposition of said complex and chromation take place, and completing the dyeing at said lowered pH.

6. A method of dyeing which comprises subjecting substantially unmetallized basic nitrogenous fibers to the action of a dye bath formed by mixing a chromable dye, a soluble chromium containing salt, magnesium sulfate, a water-dispersible surface-active composition containing at least one cationic surface active agent, water, and sufficient alkali to make the bath alkaline, but with a pH not greater than 9.5, and to cause said dye to react with said alkaline earth metal salt to form an alkaline earth metal complex of said dye and insufficient to materially damage the fibers, partially dyeing said fibers from said complex, gradually lowering the pH of said bath to a point where decomposition of said complex and chromation take place, and completing the dyeing at said lowered pH.

7. A method according to claim 1 in which the cationic surface active agent is a condensation product of octadecyl guanidine and ethylene oxide.

8. A method according to claim 2 in which the cationic surface active agent is a condensation product of octadecyl guanidine and ethylene oxide.

9. A method according to claim 4 in which the cationic surface active agent is a condensation product of octadecyl guanidine and ethylene oxide.

10. A method according to claim 6 in which the cationic surface active agent is a condensation

## 13

product of octadecyl guanidine and ethylene oxide.

HENRY E. MILLSON.  
CHESTER A. AMICK.  
WILLARD H. WATKINS.

## REFERENCES CITED

The following references are of record in the file of this patent:

## UNITED STATES PATENTS

| Number    | Name    | Date          |
|-----------|---------|---------------|
| 941,399   | Winslow | Nov. 30, 1909 |
| 1,511,359 | Onnertz | Oct. 14, 1924 |
| 2,434,178 | Royer   | Jan. 6, 1948  |

## 14

## OTHER REFERENCES

- “Theory and Practice of Wool Dyeing” by C. L. Bird, published in London in 1947 by the Society of Dyers and Colourists, pages 87, 88.
- 5 “Application of Coal Tar Dyestuffs,” by C. M. Whittaker, published in London 1919 by Balliere, Tindall and Cox, pages 59-61, inclusive.
- “Application of Dyestuffs,” by J. M. Matthews, published in New York by John Wiley & Sons, 1920. Pages 356-358.
- 10 “Metachrome Method of Dyeing,” by C. H. A. Schmitt, article in Amer. Dyes. Reporter for June 26, 1939, pages P336-P341.